# EUROPEAN PATENT SPECIFICATION

(11) **EP 3 004 298 B1**
(45) Date of publication and mention of the grant of the patent: **20.07.2022**
(21) Application number: 14728889.8
(22) Date of filing: 28.05.2014
(51) Int. Cl.: C10M 169/02, C10M 177/00, C10N 70/00, C10N 30/00, C10N 50/10, C10N 40/02

(54) **POLYMER GREASE MANUFACTURING PROCESS**
VERFAHREN ZUR HERSTELLUNG VON POLYMERFETT
PROCÉDÉ DE FABRICATION DE POLYMÈRE-GRAISSE

(30) Priority: 30.05.2013 WO PCT/EP2013/061143
(43) Date of publication of application: 13.04.2016
(73) Proprietor: Aktiebolaget SKF, 415 50 Göteborg (SE)
(72) Inventor: HOLSNIJDERS, Jos, 4142 EN Leerdam (NL); MULLER, Dries, 6531S Nijmegen (NL)
(74) Representative: Kohl, Thomas
(86) International application number: PCT/EP2014/061090
(87) International publication number: WO 2014/191470

(56) References cited:
- US-A- 2 380 893
- US-A- 2 417 495
- US-A- 2 483 282

## Description

### Technical Field

The present invention relates to the field of polymer greases and methods for the manufacture thereof.

### Background

Greases are used in a variety of engineering applications to maintain a lubricant between moving machine surfaces, such as found, for example, in bearings. A grease exhibits shear-thinning rheological properties, which means that the viscosity of the grease reduces under shear. A grease typically comprises a lubricant, such as a lubricating mineral oil, and a thickener substance. Under non-shear conditions, the thickener acts as a sponge-like matrix that holds the lubricating oil. As a result, the grease exhibits the characteristics of a solid or semi-solid. The lubricating oil may be released from the matrix both under static or dynamic conditions. In particular, when a shear force is applied, the lubricating oil separates from the thickener matrix and results in the grease exhibiting lubricating properties.

The properties of the lubricating oil are important in determining the lubricating properties of the grease. In addition, the interaction of the lubricating oil and the thickener is important in determining, for example, the longevity of a grease when used as a lubricant. In order to prolong its life as a lubricant, the oil replenishing characteristics of the grease are critical to ensure that the lubricating oil is reabsorbed into the matrix once the shear is removed from the lubricated system.

Lubricant greases for bearings are described in EP 0700986, EP 0795597 and EP 0795598. In these documents, a polymer is used as the thickener in a grease composition. The lubricating oil is chosen to be a conventional synthetic lubricating oil, such as a mineral oil, a synthetic hydrocarbon oil or an ester oil.

As described in EP 0700986, a typical method for the manufacture of a grease is to form a homogeneous mixture of the desired lubricating oil and thickener, and then to rapidly cool or quench it. This is generally achieved by pouring the composition onto a cooling table.

The present invention aims to address at least some of the problems associated with the prior art or at least to provide a commercially useful alternative thereto.

### Summary of the Invention

There is provided a process for the manufacture of a lubricating grease composition, the process comprising the steps of: providing a liquid composition comprising a mixture of lubricating oil and a thickening polymer, wherein the mixture is essentially homogenous such that it does not have any domains of separate thickening polymers within the lubricating oil or vice versa, flowing the liquid composition through a shear-mixing device to mix and cool the liquid composition to form a lubricating grease composition, wherein the thickening polymer forms from 5 to 20 wt% of the essentially homogeneous liquid composition, and wherein the liquid composition flows through the shear-mixing device along a flow-path provided with one or more temperature-controlled portions to each heat and/or cool the liquid composition, and wherein the shear-mixing device comprises one or more pairs of heat-transfer plates between which the liquid composition is flowed, wherein the surface of at least one plate is provided with surface features in the flow path of the liquid composition which are surface textures that act as baffles for the flow of the liquid composition, causing shear-mixing, wherein the essentially homogeneous liquid composition is provided at a temperature of from 150 to 350°C, preferably from 200 to 250°C.

According to a first aspect, the present invention provides a process for the manufacture of a lubricating grease composition, the process comprising the steps of:
providing an essentially homogeneous liquid composition comprising a lubricating oil and a thickening polymer;
flowing the liquid composition through a shear-mixing device to mix and cool the liquid composition to form a lubricating grease composition.

The present invention will now be further described. In the following passages different aspects of the invention are defined in more detail. Each aspect so defined may be combined with any other aspect or aspects unless clearly indicated to the contrary. In particular, any feature indicated as being preferred or advantageous may be combined with any other feature or features indicated as being preferred or advantageous.

As discussed above, conventional manufacture of polymer greases involves quenching a hot polymer/base oil mixture onto a metal plate, to room temperature. However, the present inventors have found that the grease properties (especially mechanical stability and stiffness) are extremely sensitive to the cooling process, particularly in combination with the shearing process. In particular, they have found that it is very difficult to reproduce the same grease quality due to the cooling process being a generic, uncontrolled step.

Moreover, the inventors have found that this issue affects bulk factory production to a greater extent than small-scale production. It is even more important to control and adjust cooling rates, heat dissipation, local heat distribution in the bulk, equilibrium temperatures and the like when working with larger volumes of grease. This becomes even more pronounced when producing large batches of, for example, 1-5 tons.

The present inventors found that a number of problems associated with the prior art could be addressed by using the new method disclosed herein. In particular, the method avoids pouring large production batches onto a casting table. It provides control over temperature variations, cooling rates and homogeneous heat distribution in the bulk. It further allows for the adjustment of cooling conditions to optimize grease production quality and avoids direct contact with ambient air, resulting in oxidation, contamination, and dust and particle ingress. Importantly, however, it also allows for adjustment of cooling conditions to obtain greases with different properties, either as a result of the cooling profile or because it allows the use of novel materials.

The present inventors have found that the conventional pouring-and-quenching method is not ideal for processing grease since it does not allow control of the cooling rate, or heat dissipation in the bulk material during cooling. Indeed, in contrast to the present method, such a cooling process cannot be adjusted to modify the grease properties.

By the term essentially homogeneous as used herein is meant that the components forming the liquid composition are essentially homogeneous and typically not visibly discernible in the mixture. In particular, the mixture preferably does not have any domains of the separate thickening polymers within the lubricating oils or vice versa. Preferably the liquid composition is homogeneous. Preferably the essentially homogeneous liquid composition is provided at a temperature of from 150 to 350°C, preferably from 200 to 250°C. These temperatures are generally required to ensure that the components forming the grease are thoroughly mixed and homogeneous. However, the properties of the components selected will determine the minimum temperature required to establish an essential homogeneous liquid composition.

Lubricating oils and thickening polymers are well known in the field of grease manufacture. The novel method has been found to permit a broader range of materials to be used when forming greases. Preferably the lubricating oil comprises oils selected from mineral oils, synthetic hydrocarbons, ester oils, vegetable oils, and mixtures of two or more thereof. Preferably the thickening polymer comprises a polymer selected from polyamides, polyesters, polyethylene oxides, polyethylene, polypropylene, polylactides, cellulose or cellulose derivatives, and mixtures of two or more thereof. The recited polymers are intended to encompass copolymers, as well.

The ratio of the lubricating oil and the thickening polymer helps to determine the structure of the final grease. The inventors have found that it is preferred when the thickening polymer forms from 5 to 20 wt%, preferably 9 to 15 wt% of the essentially homogeneous liquid composition. Working within this range ensures that the lubricating properties can be enhanced while providing a readily producible and stable grease product.

The liquid composition is flowed through a shear-mixing device to mix and cool the liquid composition to form a lubricating grease composition. The shear mixing device is preferably a shear-mixing conduit, preferably having a variable cross-sectional area. The use of a shear-mixing conduit is advantageous because it has contact surfaces for controlling the temperature of the liquid composition and it also allows for shear-mixing of the composition as it flows through. This is preferably achieved by the variable cross-section introducing shear into the mixture.

It is especially preferred that the shear-mixing device is a closed gas-tight system. This allows for greater control of the grease properties and it also reduces gas contamination of the lubricant. In addition, it reduces oxidation, which is an important factor if the temperature of the lubricant is increased during processing.

Preferably the liquid composition flows through the shear-mixing device along a flow-path provided with one or more static mixing elements. Static mixing elements allow for reproducible mixing. Examples of static mixers are well known in the art and include baffles, mixer bars and other obstructions in the flow-path.

Preferably the liquid composition flows through the shear-mixing device along a flow-path provided with a plurality of static mixing elements arranged to provide regions of increased shear mixing. Preferably the liquid composition flows through the shear-mixing device along a flow-path provided with one or more temperature-controlled portions to each heat or cool the liquid composition. That is, the shear-mixing device can be provided with a plurality of regions having alternative purposes. Some regions may be used to change the temperature of the lubricant flowing there-through, while others may be used to achieve high or low shear mixing. Regions may, of course, be used for temperature-control and/or shear-mixing.

It is especially preferred that at least one temperature-controlled portion is provided at a higher temperature than a preceding temperature-controlled portion along the flow-path. This allows for the heating of the lubricant after, for example, an initial cooling step. This can provide a controllable tempering or annealing step, which cannot be achieved using the conventional casting table approach. It therefore can be used to provide novel lubricants having previously unachievable properties.

In one embodiment, the shear-mixing device comprises one or more pairs of heat-transfer plates between which the liquid composition is flowed, wherein the surface of at least one plate is provided with surface features in the flow path of the liquid composition. As a consequence, the pair of plates provides both a means for raising, lowering or maintaining a temperature of the lubricant, while the surface features (on one or both of the pair of plates) can work the grease to shear-mix it. Preferably the temperature of the heat-transfer plates is controlled with water cooling. This is a cheap and effective way of controlling the temperature.

Advantageously, the lubricating grease composition can be continuously extruded using the method of the present invention. This has numerous advantages for packaging the grease compared to the conventional pouring-and-quenching method. Furthermore, it allows for greater control of the residency time of the grease within the system.

Preferably the shear-mixing is controlled by altering the flow rate of the liquid composition. This can be controlled, for example, by varying the gas pressure applied to a reservoir of the substantially homogeneous composition. To facilitate the quenching process, the flow rate may be decreased or stopped during the shear-mixing process, such that alternating dynamic and static quenching may occur.

Preferably, the shear rate and shear stress imposed on the grease are varied in the shear-mixing process such that properties of the final grease can be accurately controlled. In one embodiment, the shear rate is regulated by adjusting flow rate and geometry of the flow channels or flow plates. Especially, by narrowing the distance between plates, the shear rate can be increased to accommodate a higher shear stress and a more severe grease working process. In another embodiment, the shear stress is controlled by adjusting flow rate and temperature in each zone. Advantageously, this will enable grease working of quenched liquids of different rheological properties, in particular quenched liquids that possess a high degree of stiffness. The shear rate experienced by the homogeneous liquid during quenching, as well as during grease working, in the shear-mixing conduit, varies from 0 to 107 s⁻¹. Preferably, the thickening composition forms from shear rate varying from 10⁻¹ to 10⁵ s⁻¹. Preferably, the thickening composition forms from shear stress varying from 1 to 10⁷ Pa.

In one embodiment, one or more additives are added to the liquid composition in the shear-mixing device. These additives can be used to fine-tune the properties of the final grease.

In one embodiment, a small amount (e.g. 0.1 - 1.0%) of a co-solvent such as ethanol or water is added to the hot mixture of polymer + base oil. The co-solvent is added in order to change the solubility of the polymer in the base oil, and thus influence, e.g. the quenching temperature or thickener structure.

The process described herein provides for polymer grease synthesis whereby a hot polymer/base oil mixture is pumped through different temperature zones. This can be achieved by using a system of, for example, temperature-controlled parallel plates. These may be connected to a reactor resulting in a (semicontinuous, closed synthesis process. The polymer/base oil mixture is pumped between the plates by, for example, applying over-pressure in the reactor, resulting in a process of combined cooling and grease working. In this manner, polymer grease synthesis can be accurately controlled. In addition, conditions may be varied to adjust the properties of the polymer grease. Adjustment of cooling and grease-working may be achieved by, for example, adjusting one or more of pumping pressure and speed, gap size between the plates, shape and profile of the shape adjusted, and number of temperature zones.

The process therefore replaces the standard quenching method by combined cooling and grease working in an accurately controlled step. This allows grease synthesis with a wider range of properties and higher degree of reproducibility. The working of the grease may include shearing, straining, extrusion, rolling, forced flow and/or compression.

The invention will now be described further, by way of example, in relation to the following non-limiting figures, in which:
Figure 1 shows the microstructure of a grease composition during manufacture.
Figure 2 shows a schematic of an apparatus for use in the present invention.
Figure 3 shows a cross-section of the flow-path used in a method of the present invention.
Figure 4 shows a cooling and shear profile for the Example of the present invention.

As shown in Figure 1, the formation of a grease can occur in several steps. The four slides, A - D, show the microstructures of the grease during its formation. In slide A, the hot liquid composition (or "solution") is essentially homogeneous. In slide B, following quenching, there is a liquid-liquid separation. In slide C, there is some solidification as the thickener structure forms. With on-going working of the grease, a more stable structure is formed in slide D.

Figure 2 shows an example of an apparatus for executing the method of the invention. A reservoir is provided for the hot solution comprising the oil and the thickener as a substantially homogeneous liquid composition. The reservoir has an outlet in fluid communication with a plurality of pairs of cooling/shearing plates. The reservoir is gas-tight and in contact with a source of pressurised gas, by which the solution can be driven through the cooling/shearing plates.

As shown in Figure 2, the apparatus has three pairs of cooling/shearing plates. These each can be used to hold the liquid composition at a different temperature

(see the temperature profile in Example 1 and in Figure 4). The internal structure between the pairs of plates will determine the flow speed and the amount of shear-mixing that occurs. As shown in Figure 2, after the sequential treatment between the plates, the grease is continually extruded to fill containers for transport and sale.

As shown in Figure 3, the flow-path between pairs of parallel plates allows for working of the liquid composition. The internal surface texture of the plates acts as baffles for the flow of the liquid composition, causing shear-mixing.

Means may be provided to heat and/or cool one or more of the sets of plates. Cooling may be achieved by water-cooling. Heating may be achieved by the uses of electrical heating elements. One set of plates may comprise both cooling means and heating means.

Figure 4 shows a graph over time of the temperature (degrees Celsius) and the shear (Pa) applied in the formation of the grease in Example 1. The liquid composition of the base oil and thickener are held at a high temperature and then cooled step-wise. The shear level is controlled so that is peaks during a second quenching step. As can be seen, the shear changes stepwise as the composition moves from each set of parallel plates, but the rate of temperature change is more finely controlled, with a fast rate of cooling in the first quenching step and a slower rate at the grease is equilibrated.

### Example 1

The invention will now be described in relation to the following non-limiting example.

A homogeneous mixture was formed comprising a synthetic hydrocarbon/ester mixture as the base oil and the thickening polymer comprising a propylene polymer or co-polymer having a weight average molecular weight of from 50,000 to 100,000. This was passed through a processing unit having the following temperature and shear profile:

| **Step** | **Zone temperature** | **Shear intensity** | **Process step** |
|---|---|---|---|
| 1 | 190°C | | Homogeneous polymer/base oil solution |
| 2 | 120°C | Low shear | 1^{st} Quenching step : generation of thickener structure, determination of fiber size |
| 3 | 80 °C | High shear | 2^{nd} Quenching step : homogenisation of thickener structure |
| 4 | 25°C | Low shear | Equilibration |

The final grease had exemplary performance characteristics and was capable of continuous production.

The process as described herein is capable of improving the controllability of polymer grease synthesis. The process can be exploited to investigate the use of new polymers and/or lubricants. Furthermore, the use of a closed system allows the process to be applied beyond what is possible with current batch-production and laboratory-scale synthesis. Use of polymer types with high melting points means that temperatures for the starting mixture can be higher than temperatures currently used, which tend to be limited to a maximum of about 250°C. This allows for the development of greases with a higher temperature-limit compared to current polymer greases.

Although preferred embodiments of the invention have been described herein in detail, it will be understood by those skilled in the art that variations may be made thereto without departing from the scope of the invention or of the appended claims.

## Claims

1. A process for the manufacture of a lubricating grease composition, the process comprising the steps of:
providing a liquid composition comprising a mixture of lubricating oil and a thickening polymer, wherein the mixture is essentially homogenous such that it does not have any domains of separate thickening polymers within the lubricating oil or vice versa,
flowing the liquid composition through a shear-mixing device to mix and cool the liquid composition to form a lubricating grease composition,
wherein the thickening polymer forms from 5 to 20 wt% of the essentially homogeneous liquid composition,
and wherein the liquid composition flows through the shear-mixing device along a flow-path provided with one or more temperature-controlled portions to each heat and/or cool the liquid composition,
and wherein the shear-mixing device comprises one or more pairs of heat-transfer plates between which the liquid composition is flowed, wherein the surface of at least one plate is provided with surface features in the flow path of the liquid composition which are surface textures that act as baffles for the flow of the liquid composition, causing shear-mixing, wherein the essentially homogeneous liquid composition is provided at a temperature of from 150 to 350°C, preferably from 200 to 250°C.

2. The process according to claim 1, wherein the lubricating oil comprises oils selected from mineral oils, synthetic hydrocarbons, ester oils, vegetable oils and mixtures of two or more thereof.

3. The process according to any of the preceding claims, wherein the thickening polymer comprises a polymer selected from polyamides, polyesters, polyethylene oxides, polyethylene, polypropylene, polylactides, cellulose or cellulose derivatives, including copolymers thereof, and mixtures of two or more thereof.

4. The process according to any of the preceding claims, wherein the shear-mixing device is a shear-mixing conduit, preferably having a variable cross-sectional area.

5. The process according to any of the preceding claims, wherein the shear-mixing device is a closed gas-tight system.

6. The process according to any of the preceding claims, wherein the liquid composition flows through the shear-mixing device along a flow-path provided with one or more static mixing elements.

7. The process according to claim 6, wherein the liquid composition flows through the shear-mixing device along a flow-path provided with a plurality of static mixing elements arranged to provide regions of increased shear mixing.

8. The process according to any of the preceding claims, wherein at least one of the temperature-controlled portions is at a higher temperature than a preceding temperature-controlled portion along the flow-path.

9. The process according to any of the preceding claims, wherein the temperature of the heat-transfer plates is controlled with water cooling.

10. The process according to any of the preceding claims, wherein the lubricating grease composition is continuously extruded.

11. The process according to any of the preceding claims, wherein the shear-mixing is controlled by altering the flow rate of the liquid composition.

12. The process according to any of the preceding claims, wherein one or more additives are added to the liquid composition in the shear-mixing device.

## Patentansprüche

1. Verfahren zur Herstellung einer Schmierfettzusammensetzung, das Verfahren die folgenden Schritte umfassend:
Bereitstellen einer flüssigen Zusammensetzung, die eine Mischung aus Schmieröl und einem verdickenden Polymer enthält, wobei die Mischung im Wesentlichen homogen ist, so dass sie keine Domänen separater verdickender Polymere in dem Schmieröl oder vice versa aufweist,
Strömen der flüssigen Zusammensetzung durch eine Scherungsmischvorrichtung, um die flüssige Zusammensetzung zu mischen und abzukühlen, um eine Schmierfettzusammensetzung auszubilden,
wobei das verdickende Polymer zwischen 5 und 20 Masse-% der im Wesentlichen homogenen flüssigen Zusammensetzung ausbildet
und wobei die flüssige Zusammensetzung entlang eines Strömungswegs durch die Scherungsmischvorrichtung strömt, der mit einem oder mehreren temperaturgeregelten Abschnitten versehen ist, um die flüssige Zusammensetzung jeweils zu erwärmen und/oder abzukühlen
und wobei die Scherungsmischvorrichtung ein oder mehrere Paare Wärmetransferplatten umfasst, zwischen denen die flüssige Zusammensetzung strömt, wobei die Oberfläche mindestens einer Platte in dem Strömungsweg der flüssigen Zusammensetzung mit Oberflächenmerkmalen versehen ist, die Oberflächentexturen sind, die für die Strömung der flüssigen Zusammensetzung als Prallflächen wirken, die ein Scherungsmischen bewirken, wobei die im Wesentlichen homogene flüssige Zusammensetzung bei einer Temperatur zwischen 150 und 350 °C, vorzugsweise zwischen 200 und 250 °C, bereitgestellt wird.

2. Verfahren nach Anspruch 1, wobei das Schmieröl Öle enthält, die aus Mineralölen, synthetischen Kohlenwasserstoffen, Esterölen, Pflanzenölen und Mischungen aus mindestens zwei von diesen ausgewählt sind.

3. Verfahren nach einem der vorhergehenden Ansprüche, wobei das verdickende Polymer ein Polymer enthält, das aus Polyamiden, Polyestern, Polyethylenoxiden, Polyethylen, Polypropylen, Polylactiden, Cellulose oder Cellulose-Derivaten, einschließlich ihrer Copolymere, und Mischungen aus mindestens zwei von diesen ausgewählt ist.

4. Verfahren nach einem der vorhergehenden Ansprüche, wobei die Scherungsmischvorrichtung eine Scherungsmischröhre, vorzugsweise mit einer variablen Querschnittsfläche, ist.

5. Verfahren nach einem der vorhergehenden Ansprüche, wobei die Scherungsmischvorrichtung ein geschlossenes gasdichtes System ist.

6. Verfahren nach einem der vorhergehenden Ansprüche, wobei die flüssige Zusammensetzung entlang eines Strömungswegs durch die Scherungsmischvorrichtung strömt, der mit einem oder mehreren statischen Mischelementen versehen ist.

7. Verfahren nach Anspruch 6, wobei die flüssige Zusammensetzung entlang eines Strömungswegs durch die Scherungsmischvorrichtung strömt, der mit mehreren statischen Mischelementen versehen ist, die eingerichtet sind, um Bereiche erhöhter Scherungsmischung bereitzustellen.

8. Verfahren nach einem der vorhergehenden Ansprüche, wobei mindestens einer der temperaturgeregelten Abschnitte bei einer höheren Temperatur ist als ein entlang des Strömungswegs vorhergehender temperaturgeregelter Abschnitt.

9. Verfahren nach einem der vorhergehenden Ansprüche, wobei die Temperatur der Wärmetransferplatten durch Wasserkühlung geregelt wird.

10. Verfahren nach einem der vorhergehenden Ansprüche, wobei die Schmierfettzusammensetzung kontinuierlich extrudiert wird.

11. Verfahren nach einem der vorhergehenden Ansprüche, wobei das Scherungsmischen durch Verändern der Strömungsrate der flüssigen Zusammensetzung geregelt wird.

12. Verfahren nach einem der vorhergehenden Ansprüche, wobei in der Scherungsmischvorrichtung ein oder mehrere Zusatzstoffe zu der flüssigen Zusammensetzung hinzugefügt werden.

## Revendications

1. Procédé pour la fabrication d'une composition de graisse lubrifiante, le procédé comprenant les étapes suivantes :
la fourniture d'une composition liquide comprenant un mélange d'une huile lubrifiante et d'un polymère épaississant, dans lequel le mélange est pratiquement homogène de telle sorte qu'il ne présente pas de domaines de polymères épaississants séparés dans l'huile lubrifiante ou vice versa,
l'écoulement de la composition liquide à travers un dispositif de mélange par cisaillement pour mélanger et refroidir la composition liquide afin de former une composition de graisse lubrifiante,
dans lequel le polymère épaississant forme de 5 à 20 % en poids de la composition liquide pratiquement homogène,
et dans lequel la composition liquide s'écoule à travers le dispositif de mélange par cisaillement le long d'un chemin d'écoulement pourvu d'une ou de plusieurs parties à température contrôlée pour chauffer et/ou refroidir chacune la composition liquide,
et dans lequel le dispositif de mélange par cisaillement comprend une ou plusieurs paires de plaques de transfert de chaleur entre lesquelles la composition liquide s'écoule, dans lequel la surface d'au moins une plaque est pourvue d'éléments de surface dans le chemin d'écoulement de la composition liquide qui sont des textures de surface qui font office de chicanes pour l'écoulement de la composition liquide, provoquant un mélange par cisaillement, dans lequel la composition liquide pratiquement homogène est fournie à une température de 150 à 350 °C, de préférence de 200 à 250 °C.

2. Procédé selon la revendication 1, dans lequel l'huile lubrifiante comprend des huiles choisies parmi des huiles minérales, des hydrocarbures de synthèse, des huiles d'esters, des huiles végétales et des mélanges de deux ou plusieurs de ceux-ci.

3. Procédé selon l'une quelconque des revendications précédentes, dans lequel le polymère épaississant comprend un polymère choisi parmi des polyamides, des polyesters, des oxydes de polyéthylène, du polyéthylène, du polypropylène, des polylactides, de la cellulose ou des dérivés de cellulose, notamment des copolymères de ceux-ci, et des mélanges de deux ou plusieurs de ceux-ci.

4. Procédé selon l'une quelconque des revendications précédentes, dans lequel le dispositif de mélange par cisaillement est un conduit de mélange par cisaillement, de préférence ayant une aire en coupe transversale variable.

5. Procédé selon l'une quelconque des revendications précédentes, dans lequel le dispositif de mélange par cisaillement est un système fermé étanche aux gaz.

6. Procédé selon l'une quelconque des revendications précédentes, dans lequel la composition liquide s'écoule à travers le dispositif de mélange par cisaillement le long d'un chemin d'écoulement pourvu d'un ou de plusieurs éléments de mélange statiques.

7. Procédé selon la revendication 6, dans lequel la composition liquide s'écoule à travers le dispositif de mélange par cisaillement le long d'un chemin d'écoulement pourvu d'une pluralité d'éléments de mélange statiques disposés pour fournir des régions de mélange par cisaillement accru.

8. Procédé selon l'une quelconque des revendications précédentes, dans lequel au moins une des parties à température contrôlée est à une température plus élevée qu'une partie à température contrôlée précédente le long du chemin d'écoulement.

9. Procédé selon l'une quelconque des revendications précédentes, dans lequel la température des plaques de transfert de chaleur est contrôlée avec un refroidissement à l'eau.

10. Procédé selon l'une quelconque des revendications précédentes, dans lequel la composition de graisse lubrifiante est extrudée en continu.

11. Procédé selon l'une quelconque des revendications précédentes, dans lequel le mélange par cisaillement est contrôlé en modifiant le débit de la composition liquide.

12. Procédé selon l'une quelconque des revendications précédentes, dans lequel un ou plusieurs additifs sont ajoutés à la composition liquide dans le dispositif de mélange par cisaillement.
